

June 19, 1945.

F. E. FREY

2,378,763

## MAKING LUBRICATING OIL CONSTITUENTS

Original Filed Dec. 4, 1942



## UNITED STATES PATENT OFFICE

2,378,763

## MAKING LUBRICATING OIL CONSTITUENTS

Frederick E. Frey, Bartlesville, Okla., assignor to  
 Phillips Petroleum Company, a corporation of  
 Delaware

Original application December 4, 1942, Serial No.  
 467,875. Divided and this application October  
 4, 1943, Serial No. 504,944

8 Claims. (Cl. 196—78)

This invention relates to the treatment of hydrocarbons. More particularly it relates to the improvement of lubricating oil stocks by treatment with concentrated hydrofluoric acid.

Lubricating oils of high quality have been manufactured from crude oil fractions having suitable boiling ranges by many processes, including sulfuric acid refining, aluminum chloride refining, and solvent extraction. In sulfuric acid or aluminum chloride processes, the treating reagents are consumed by reaction with the oil and are not economically recoverable from the resulting sludges. In solvent refining, the action is simply one of separating high-quality lubricating ingredients from the crude oil, or removing the undesirable or low-quality constituents; thus the yield of finished lubricating oil can be no greater than the proportion of lubricating oil-grade hydrocarbons in the raw material.

An object of this invention is to produce high-quality lubricating oil in high yield by a chemical process in which the chemical reagent is recoverable.

Another object of this invention is to convert paraffin wax to normally liquid hydrocarbons suitable for blending in lubricating oil.

Another object of this invention is to improve cyclic materials for use as ingredients in lubricating oil.

Another object is to combine advantageously, into a process for manufacturing lubricating oil, steps for treating oil stocks with hydrofluoric acid with steps for solvent refining of the oil stocks.

Other objects and advantages of this invention will be apparent to those skilled in the art from the following description, the accompanying drawing, and/or the appended claims.

According to this invention, a lubricating oil stock is treated with concentrated or substantially anhydrous liquid hydrofluoric acid under conditions selected to improve or modify the properties of the oil. Properties which may be changed include one or more of the following: viscosity or viscosity index, flash and fire points, pour point, and carbon residue. These changes are preferentially promoted by carrying out the reaction in the presence of solvents or diluents such as low-boiling normally liquid hydrocarbons or halogenated hydrocarbons, in the presence of added alkylating agents, such as olefins or polymers of olefins having 2 to 5 carbon atoms per molecule, or in the presence of catalyst modifiers, such as boron fluoride, sulfur trioxide, phosphoric anhydride, halides of antimony, arsenic or bismuth, or dissolved salts or colloidal suspensions

of the following metals: silver, nickel, cobalt, chromium, tin, zirconium, or other metals selected from the third and fourth periods of the periodic table.

- 5 The exact nature of the chemical changes which occur in the treatment are not known. It is presumed that a number of reactions occur simultaneously and that the nature and the extent of the predominating reactions are influenced appreciably by varying the conditions of temperature and pressure and by the use of solvents, alkylating agents, catalyst modifiers, and the like. As disclosed in my copending application, Ser. No. 426,627, filed January 13, 1942, paraffinic hydrocarbons in the presence of concentrated hydrofluoric acid undergo extensive reconstruction to lower- and higher-boiling hydrocarbons and also to one or more hydrocarbons having the same number of carbon atoms but 10 different carbon-skeletal structure. Alkylation probably occurs to some extent if alkylating agents are present in the reaction mixture, particularly when aromatic ring compounds are present as components in the oil being treated. High-boiling olefinic hydrocarbons may undergo reactions such as cyclization to naphthenes, depolymerization, isomerization, or disproportionation to paraffins and diolefins or aromatics. Aromatics may undergo condensation reactions 15 with added alkylating agents, such as ethylene, propylene, halogenated hydrocarbons, alcohols, and the like. Sulfur, nitrogen, and oxygen compounds in the lubricating oil may be simultaneously removed by absorption in, or formation of loose compounds with, the hydrofluoric acid. The presence of boron fluoride, sulfur trioxide, phosphoric anhydride, or the like, appears to increase the catalytic activity and the selective solvent power of the hydrofluoric acid. Boron fluoride is particularly effective when in concentration of 1 to 5 per cent. The nature of the effects is also dependent upon the nature of the lubricating feed stock.
- 20 Treatment of lubricating oil stocks with hydrofluoric acid under relatively mild conditions of temperature and time, such as 50 to 250° F. and for a time of 1 to 30 minutes, ordinarily raises the viscosity index, increases the API gravity slightly, improves the color, and raises the pour point slightly; it usually does not change the absolute viscosity greatly. Under relatively drastic conditions, such as at a temperature in the range of 300 to 450° F., or with a contact time of one 25 or more hours, the absolute viscosity decreases 30 substantially. The extent of reaction is con-
- 35
- 40
- 45
- 50
- 55

trollable to some degree by limiting the proportion of hydrofluoric acid used in the treatment. That is, hydrogen fluoride tends to form molecular complexes and addition compounds with some of the more reactive or less stable hydrocarbons found in lubricating oil, and if the proportion of hydrofluoric acid is limited, say to from 5 to about 50 per cent by weight of the lubricating oil being treated, the reaction slows down or stops after the more reactive constituents have been removed by reaction with the acid. A low-temperature process may be controlled in this manner to produce results similar to those obtained by solvent refining.

Crude lubricating oil stocks vary widely in composition. The various components may be classified in the following groups:

|                          |
|--------------------------|
| Asphalt                  |
| Resins                   |
| Naphthenes               |
| Cyclo-alkyl compounds    |
| Paraffins, including wax |
| Color bodies             |

Asphaltic constituents are tarry or pitchy materials of aromatic structure. Resins are similar but of lower molecular weight and more soluble in paraffin hydrocarbons. These constituents cause sludge and varnish formation in motor oils, and therefore must be removed by oil-refining processes.

By naphthenes is meant saturated liquid hydrocarbons which are predominantly cyclic in structure. Such hydrocarbons have good lubricating properties for use at constant temperatures, but the viscosity index is low; that is, the viscosity varies greatly with the temperature. Consequently, only a limited proportion may be present in lubricating oil of high viscosity index.

The cyclo-alkyl compounds are hydrocarbons having one or more cyclic nuclei with long aliphatic chains attached thereto. These compounds are the preferred predominant constituents of lubricating motor-oils for general use. The viscosity index is high; the pour point is low; the carbon-forming tendency is low; and the oils are stable against oxidation.

The paraffins have very high viscosity indices, and good lubricating properties. However, the carbon-forming tendency is greater than for cyclo-alkyl compounds. As many of the paraffins present in lubricating oil stocks have high melting points, the proportion of paraffins which may be present in the final lubricating oil is limited mainly by the maximum permissible pour point of the oil. The allowable proportion of paraffins may be increased somewhat by using pour point depressants.

The structure of the color bodies is not fully known. They are objectionable mainly because of consumer demand for oil of clear and standard appearance.

Concentrated hydrofluoric acid has both a solvent effect and a chemical effect upon the lubricating oil. By its solvent effect, it dissolves asphaltic, resin-forming, and other cyclic hydrocarbons preferentially to cycloalkyl and paraffinic hydrocarbons. The extent of the solvent effect is dependent upon the temperature, the pressure, the proportion of hydrofluoric acid, and the presence or absence of another solvent. For example, at room temperature, asphaltic, aromatic, unsaturated, and naphthenic hydrocarbons are appreciably soluble in concentrated hydrofluoric acid, whereas paraffinic and cycloalkyl hydrocar-

bons, or hydrocarbons of high hydrogen-to-carbon ratios, are substantially insoluble. As the temperature is increased, the solvent power of concentrated hydrofluoric acid increases until at about 350° F. and two thousand pounds per square inch pressure the acid is almost completely miscible with cycloalkyl hydrocarbons. Thus concentrated hydrofluoric acid may be used similarly to a single solvent in a series of solvent extraction steps at progressively higher temperatures to "fractionate" lubricating oil stocks into extracts of progressively increasing "paraffinicity" or hydrogen-to-carbon ratio. There are always some chemical reconstruction reactions of the more reactive of the ingredients, though if desired these may be retarded by the use of short contact times.

The efficiency of the extraction of cycloalkyl hydrocarbons from lube oil stock by concentrated hydrofluoric acid may be greatly increased by concurrently using a "deasphalting" diluent or selective solvent which is immiscible with hydrofluoric acid. Liquid propane is a preferred diluent. That is, at temperatures in the range of about 50 to 200° F., propane dissolves paraffins and cycloalkyl hydrocarbons in lubricating oil, but precipitates substantial proportions of asphaltic and resinous materials. Thus the use of propane as a diluent for treating lube oil stocks with hydrofluoric acid greatly increases the selective solvent power of the acid for removing asphaltic, resinous, and aromatic constituents from the oil. Other low-boiling hydrocarbons such as ethane, butane, pentanes, or mixtures are also advantageous in some instances. For example, in carrying out the treatment at high temperatures such as 200 to 450° F., butane, pentanes, or even higher-boiling paraffins are advantageous because lower pressures may be used than with propane. Next to propane, butane is preferred.

The chemical effect of hydrofluoric acid on asphaltic constituents appears to be slight. Resin-forming substances are probably condensed to form resins and asphaltic compounds. Aromatics and naphthenes appear to be substantially unaffected except in the presence of alkylating agents or under drastic conditions of time and temperature. In the presence of alkylating agents, they appear to be converted in part to compounds of greater "paraffinicity," presumably by addition of aliphatic side chains to the cyclic structures. At high temperatures some of the cycloalkyl hydrocarbons and corresponding lower-molecular-weight paraffins appear to be comparatively stable and unaffected by hydrofluoric acid, although some molecular rearrangements may occur at high temperatures. Paraffins are broken down to lower-molecular-weight compounds in high-temperature treatments, and if low-molecular-weight aromatics, such as benzene or naphthalene, are present, alkyl aromatics may be formed in appreciable proportions.

The treatment given a specific lubricating oil stock depends in large measure upon the nature of the stock. Paraffin-base crudes, such as are found in Pennsylvania oils, require a treatment which removes paraffin wax or converts part of it to lower-melting materials; that is, the pour point of the oil must be decreased by the refining process. Asphalt-base crudes, such as are found in California and along the Gulf Coast, require a treatment which removes asphaltic, resinous,

and naphthenic components or converts them to materials of relatively higher paraffinicity or hydrogen-to-carbon ratio; that is, the viscosity index of the oil must be increased. Mixed-base crudes, such as are found in Oklahoma, Kansas, and Illinois, require treatment to remove unstable easily oxidizable or varnish-forming constituents and to modify the pour point and viscosity index.

In treating paraffin-base crudes according to the principles of this invention, it is usually desirable to add some unsaturated cyclic materials, such as benzene, terpenes, and the like, to the oil prior to or during contacting with hydrofluoric acid. The added cyclic compounds react in the presence of hydrofluoric acid with part of the high-molecular-weight paraffins or waxes of the oil to produce highly desirable cyclo-alkyl compounds and paraffins of relatively low molecular weight. This decreases the pour point of the oil without excessively decreasing the viscosity index and produces a maximum yield of refined lubricating oil.

In treating asphalt-base crudes according to the principles of this invention, it is desirable to add aliphatic alkylating agents, such as olefins, cracked gasoline, alcohols, or alkyl halides, to the oil prior to or during contacting with hydrofluoric acid. The added alkylating agents react in the presence of hydrofluoric acid with naphthenic and aromatic constituents of the oil to produce compounds of increased paraffinicity or hydrogen-to-carbon ratio. This increases the viscosity index of the oil and gives a much higher yield of refined oil than solvent extraction methods, which simply remove naphthenic components from the crude oil.

In treating mixed-base crudes, it may sometimes be desirable to add alkylating agents, depending upon whether the properties of the specific crude treated approach those of paraffin-base crudes or of asphalt-base crudes. In general, a simple treatment with hydrofluoric acid in the presence of a solvent, followed by a decolorizing, and in some cases a dewaxing, step gives very satisfactory results.

Understanding of some aspects of my invention may be aided by referring to the accompanying drawing, which is a schematic flow diagram of one preferred arrangement of apparatus for practicing my invention. In this specific embodiment of my invention, propane is used to dilute the lubricating oil and to aid the acid in separating asphalt and wax from the oil. In some instances it is desirable to use an isoparaffin such as isobutane or isopentane, for such isoparaffins at relatively low temperatures will react with unsaturates in the oil in the presence of hydrofluoric acid to produce saturates and at relatively high temperatures will react with high-melting paraffins to produce relatively low-melting paraffins.

Liquid propane and crude lubricating oils are admitted, as through inlets 10 and 11, respectively, to mixer 12, in which they are mixed together at a deasphalting temperature. In some modifications of this invention, especially for treating paraffin-base crudes, it will be desirable to use a cyclic hydrocarbon, such as benzene, as the solvent or as one component of the solvent; for treating most mixed-base and asphalt-base crudes, low-boiling paraffins, such as liquid propane, appear to be the most suitable solvents. One distinct advantage in using propane as the solvent results from the fact that hydrogen fluoride is soluble in liquid propane to the extent

of several per cent at temperatures only slightly above room temperature. This facilitates contacting of the oil with the acid. The optimum temperature depends to some extent upon the nature of the feed stock but is usually in the range of about 50 to 200° F. In general, asphaltic and resinous constituents are less soluble in propane at high temperatures than at low. The pressure should be sufficient to maintain substantially all the propane in the liquid phase and will generally be in the range of 100 to 600 pounds per square inch or more. The propane-to-oil ratio may range from 2:1 to 10:1 by weight. Generally a ratio in the range of 2.5:1 to 5:1 is preferred. At lower ratios the diluting and deasphalting action of propane is relatively inefficient, whereas at higher ratios the quantity of propane being handled may be excessive. Under the preferred conditions mentioned, propane dissolves substantially all of the lubricating oil constituents except asphaltic and resinous substances.

From mixer 12 the mixture passes to asphalt settler 13, wherein asphaltic and resinous materials settle out and are removed through outlet 14. The temperature may be reduced somewhat in settler 13 by allowing part of the propane to evaporate and to be removed as vapor through conduit 15.

From settler 13 the resulting deasphalting mixture is transferred by pump 16 through conduit 17 to treater 18. In treater 18 it is agitated with concentrated or substantially anhydrous hydrofluoric acid which may be introduced through inlet 19 and/or recycle conduits 20 and 21. Treater 18 may be operated at a temperature in the range of about 50 to about 450° F. The exact temperature chosen in a particular instance will depend upon the characteristics of the crude oil, the solvent effect desired, the chemical effect desired, and the proportion of hydrofluoric acid used. In most instances the preferred temperature is in the range of 100 to 300° F. In general, at the lower temperatures within the operative range, unstable constituents such as unsaturated compounds, organic acids, resin- or sludge-forming materials are extracted by solution in the hydrofluoric acid; in the absence of alkylating agents, the other constituents may undergo some molecular rearrangement and reconstruction reactions but, as a whole, are not greatly changed. If an alkylating agent, such as an olefin, a nonprimary alkyl halide, or a non-primary alcohol, is present, considerable reaction occurs, and the yield of lubricating oil may be greatly increased. The alkylating agent appears to react preferentially with cyclic compounds and with cyclic groups in cyclo-alkyl compounds, thereby increasing the "paraffinicity" or hydrogen-to-carbon ratio of these compounds, reducing their solubility in hydrofluoric acid, and rendering them more suitable as constituents in lubricating oil.

At the higher temperatures within the operative range, hydrofluoric acid in large proportions extracts substantially all of the aromatic compounds and considerable proportions of the non-aromatic cyclic compounds. It may also cause extensive chemical reconstruction of the remaining compounds if the reaction time is sufficiently long. Part of the aliphatics or waxes are converted to compounds of lower molecular weight. Waxes may react with low-boiling aromatics, such as benzene, naphthalene, anthracene, and the like, to produce normally liquid alkyl aro-

matics, which act to decrease the pour point of the lubricating oil. For this reason it is advantageous in some instances, for example when the crude oil contains relatively large proportions of wax or has a relatively high pour point, to add a low-boiling aromatic to the reaction mixture. At temperatures above about 200° F., ethylene, primary alcohols, and primary alkyl halides may be used as alkylating agents.

The proportion of hydrofluoric acid in the mixture may vary from about 0.1 to 10 parts or more by weight per part of the crude oil, depending upon the nature of the crude oil and the desired characteristics of the refined oil. For producing high-grade motor lubricating oils from average lubricating oil stock, the optimum proportion of acid usually is in the range of about 0.5 to 4 parts by weight per part of the crude oil. By treating the oil with several relatively small successive portions of hydrofluoric acid, the effect is substantially that of a selective solvent; that is, the relatively unstable compounds form complexes with the acid which dissolve in the acid phase, and the relatively stable constituents are substantially unaffected. When a large excess of hydrofluoric acid over that required to tie up or remove, as compounds or molecular complexes, most of the unstable or undesired constituents is used, and when a sufficient reaction time is allowed, the relatively stable acid-insoluble lubricating oil constituents undergo considerable chemical change as already described.

The reacted mixture from treater 18 is passed through conduit 22 to cooler 23, wherein by flash evaporation of part of the propane and hydrogen fluoride from the mixture, the remainder is cooled to the desired separating temperature. The separating temperature determines the extent of the solvent action of the acid. The optimum temperature is usually in the range of 50 to 300° F. though at times it may exceed this range in either direction. At low temperatures, such as 50° F., only the unsaturated compounds, aromatics, and nitrogen-, sulfur-, and oxygen-containing compounds dissolve appreciably in the acid. At high temperatures, such as 300° F. and above, substantially all aromatics and substantial proportions of nonaromatic cyclic compounds are extracted by, and removed in, the acid phase.

Vapors from cooler 23 are condensed and recycled through conduit 24 and pump 25 to treater 18. Liquids are passed through conduit 26 to separator 27, wherein they are separated by centrifugal or gravitational means at the desired separating temperature into two liquid phases. In instances when only a relatively minor proportion of hydrogen fluoride is used in treater 18, separator 27, may be by-passed—all hydrogen fluoride being flashed or distilled overhead and recycled from cooler 23 and/or fractionator 29.

The upper or hydrocarbon phase from separator 27 is passed through conduit 28 to fractionating column 29. Substantially all the dissolved hydrogen fluoride in the mixture is withdrawn as an overhead azeotropic mixture of propane and hydrofluoric acid and is condensed and recycled through conduit 24 and pump 25 to reactor 18.

The resulting hydrogen fluoride-free hydrocarbon mixture is passed through conduit 30 to deasphalting unit 31. The deasphalting unit consists essentially of a means for adjusting the temperature of the propane-hydrocarbon mixture and allowing the asphalt to settle out. The deasphalt-

ing temperature may be in the range of about 70 to 200° F. depending upon the degree of deasphalting desired. Asphaltic and resinous substances may be withdrawn through outlet 32, and the deasphalted hydrocarbon mixture is passed through conduit 33 to dewaxing unit 34.

In dewaxing unit 34, the propane-oil solution is chilled slowly to a temperature in the range of about -50 to 70° F., whereupon wax crystallizes out. The wax is then removed by known means, such as centrifugation or filtration. The purpose of dewaxing is mainly to reduce the pour point of the oil to a desired value. Experience has shown that, in order to obtain an oil of given pour point, the dewaxing temperature should be in the range of about 20 to 40° F. below the desired pour point. In order to obtain an easily separable wax, the chilling rate should not be more than about 3° F. per minute. Filter-aids may be added if desired. Cooling of the mixture is effected by evaporation of part of the propane, which may be recycled, as through conduit 35 and pump 36 to mixer 12. Wax may be withdrawn through outlet 37. The dewaxed oil is passed through conduit 38 to decolorizer 39, in which it is subjected at a suitable temperature to the action of a contact mass having catalytic properties for hydrogenation and/or dehydrogenation at relatively higher temperatures, such as finely divided nickel, bauxite, etc.

Decolorizer 39 may consist of a conventional bauxite or clay treater such as is well-known in the art of refining lubricating oil. Preferably it is a bauxite filter bed. The propane-oil mixture is allowed to percolate through the bauxite at a temperature in the range of about 50 to 500° F. The most efficient decolorization usually occurs at temperatures in the range of 150 to 300° F. In the decolorizing step, organically combined fluorine is also substantially completely removed.

The resulting clear, fluorine-free, dewaxed, and deasphalted propane-oil mixture is passed through conduit 40 to depropanizer 41. In depropanizer 41 the oil is freed from propane by distillation; the propane is recycled through conduits 42 and 35 and pump 36 to mixer 12. Lubricating oil of high viscosity index, low pour point, and low carbon-forming qualities is withdrawn through outlet 43. If desired, it may be fractionated, as by vacuum distillation, into several cuts of different viscosity, or it may be blended with other oils to modify its properties.

The heavier or acid layer from separator 27 may be recycled in part through conduit 21 to treater 18; preferably a substantial proportion is passed through conduit 44 to column 45, and a proportion of about 1 to 5 times the weight of wax available for the presently described conversion to a pour point depressant is passed through conduit 46 to reactor 47.

In reactor 47 petroleum wax, such as that produced in dewaxing unit 34, is agitated with substantially anhydrous hydrofluoric acid (such as the used acid from separator 27) and one or more unsaturated or aromatic compounds, such as benzene, naphthalene, alkyl benzenes, alkyl naphthalenes, cycloolefins, terpenes, and the like, added through inlet 62. The temperature may be from about 150 to about 450° F. Preferably it is in the range of 250 to 350° F. At low temperatures the rate of reaction is low, whereas at high temperatures excessive cracking occurs. The mixture should be continuously agitated to insure intimate contacting and to prevent separation of

phases. The pressure should be sufficient to maintain liquid- or mixed-phase conditions; usually it will be in the range of about 50 to 2000 pounds per square inch. The contact time may vary from 1 to 100 minutes or more. The optimum contact time varies inversely with the temperature. Under these conditions petroleum waxes, such as those obtained from lubricating oil fractions, react with low-molecular-weight cyclic compounds having double bonds, such as aromatics, cycloolefins, terpenes, and the like, to produce cyclo-alkyl compounds, consisting of cyclic nuclei with one or more attached alkyl groups, and paraffins of a molecular weight lower than that of the original wax. If desired a diluent or solvent, such as light naphtha or propane, may be used in reactor 47 to reduce the viscosity of the mixture and to facilitate handling it.

The mixture from reactor 47 passes through conduit 48 to separator 49, in which it is separated, by cooling and centrifugal or gravitational means, into two liquid phases. The lighter or hydrocarbon phase is passed through conduit 50 to fractionator 51. From fractionator 51 an overhead fraction, comprising unreacted low-molecular-weight reactants, diluent or solvent, and hydrogen fluoride, is recycled via conduit 52 to reactor 47. The bottom fraction, which consists mainly of cyclo-alkyl hydrocarbons having long alkyl groups, is withdrawn through outlet 53. This fraction is suitable for use as a pour-point depressant in lubricating oils.

The lower or acid layer from separator 49 is passed through conduit 54 to column 45. Column 45 is operated with a high enough kettle bottom temperature, preferably in the range 300 to 500° F., to split out substantially all organically combined fluorine as hydrogen fluoride. This hydrogen fluoride, any water incidentally introduced into the process, and a substantial proportion of the hydrocarbons present pass overhead through conduit 55 to column 56. A high-boiling residue oil is withdrawn through outlet 57.

Column 56 separates hydrofluoric acid and water, which passes overhead through conduit 58 to acid-rerun column 59, from hydrocarbons, which may be withdrawn through outlet 60. These hydrocarbons are liquid, of a clear color, have a low pour point, and are suitable for blending in small proportions with other lubricants.

Column 59 separates a constant-boiling mixture of water and hydrogen fluoride, which may be withdrawn through outlet 61, from substantially anhydrous hydrogen fluoride, which is recycled through conduit 20 to treater 18.

To further illustrate some of the many aspects of this invention the following specific example is given:

*Example I*

To a steel reactor having a mechanical stirrer were charged 0.48 pounds of a mixed-base lubricating oil, 2.09 pounds of substantially pure hydrogen fluoride, and 0.75 pound of normal pentane. The mixture was agitated for one hour at 185° F. and then was separated into two phases. The hydrocarbon phase was washed free of hydrogen fluoride and was topped to 293° F., chiefly to remove the pentane. The remaining hydrocarbon was equivalent to 84.8 per cent by weight of the original oil. Part of this material was tested by conventional lubricating oil tests. Another part was clay-treated by agitating it with fuller's earth and filtering; it was then also tested

by conventional lubricating oil tests. The following test data were obtained:

|                          |                                  | Untreated oil | HF treated | HF+ clay treated |
|--------------------------|----------------------------------|---------------|------------|------------------|
| 5                        | Viscosity, S. U. V.:             |               |            |                  |
| 100° F.                  | 469                              | 427           | 413        | 57.7             |
| 210° F.                  | 58.8                             | 58.3          |            |                  |
| 10                       | Viscosity index (Dean and Davis) | 81            | 90.5       | 91               |
| Carbon residue, per cent | 0.24                             | 0.28          | 0.18       |                  |
| Color, N. P. A.          | 5                                | Dark          |            | 31/4             |
| Gravity, A. P. I.        | 26.2                             | 27.9          | 27.8       |                  |
| Aniline No., °F.         | 213                              |               | 222        |                  |
| Pour point, °F.          | -5                               |               | +10        |                  |

15 From these data it is evident that the treatment increased the viscosity index of the oil, reduced the carbon-forming tendencies, and improved the color. The increase in pour point indicates an increase in paraffin content and a corresponding decrease in naphthenes.

20 This invention is broadly applicable to many modified processes for refining oils. It may be applied to the refining of various grades of crude oil, including paraffin-base crudes, mixed-base crudes, and asphalt-base crudes. It may be used for producing any grade of oil, including such highly refined oils as transformer oil. It may be used advantageously in combination with older methods of refining, such as solvent refining and sulfuric acid refining. It may be particularly advantageously combined with propane de-asphalting and dewaxing steps, whereby the propane also serves as a diluent in steps for treating the oil with hydrofluoric acid. It may be used in conjunction with alkylating agents to change appreciably the chemical constitution of the oil. Further, highly paraffinic lubricating oil fractions, such as petroleum waxes, may be converted in the presence of concentrated hydrofluoric acid and cyclic hydrocarbons to hydrocarbons of lower pour point and better adaptability for use as constituents in lubricating oil.

25 30 35 40 45 50 Because the invention may be practiced otherwise than as specifically described or illustrated, and because many modifications and variations within the spirit and scope of it will be obvious to those skilled in the art of treating lubricating oil stocks, the invention should not be unduly restricted by the foregoing specification and illustrative example, but it should be restricted only in accordance with the appended claims.

55 This application is a division of my copending application, Serial No. 467,875, filed December 4, 1942, which in turn is a continuation-in-part of my copending application, Serial No. 426,627, filed January 13, 1942.

I claim:

1. The process of manufacturing lubricating oil constituents which comprises reacting paraffin wax as such with a normally liquid cyclic hydrocarbon having at least one double bond in the ring in the presence of substantially anhydrous hydrofluoric acid at an elevated temperature and at a pressure sufficient to maintain liquid phase conditions.
2. The process of claim 1 in which the substantially anhydrous hydrofluoric acid is used acid from refining crude lubricating oil with hydrofluoric acid.
3. The process of claim 1, in which said cyclic hydrocarbon is benzene.
4. The process of making lubricating oil constituents which comprises reacting paraffin wax as such with a normally liquid cyclic hydrocarbon having at least one double bond in the ring by means of substantially anhydrous hydrofluoric

acid at a temperature ranging from 150 to 450° F. and at a pressure sufficient to maintain liquid phase conditions.

5. The process of making lubricating oil constituents which comprises reacting paraffin wax as such with a normally liquid cyclic hydrocarbon having at least one double bond in the ring by means of substantially anhydrous hydrofluoric acid at a temperature ranging from 250 to 350° F. and at a pressure sufficient to maintain liquid phase conditions.

6. The process of making lubricating oil constituents which comprises reacting paraffin wax as such with benzene by means of substantially anhydrous hydrofluoric acid at a temperature ranging from 250 to 350° F. and under a pressure sufficient to maintain liquid phase conditions.

7. The process of making lubricating oil constituents which comprises reacting paraffin wax as such with naphthalene by means of substantially anhydrous hydrofluoric acid at a temperature ranging from 250 to 350° F. and under a

pressure sufficient to maintain liquid phase conditions.

8. The process of making a material suitable for use as a pour-point depressant in lubricating oils which comprises reacting paraffin wax as such with a low-molecular weight cyclic hydrocarbon having at least one double bond by means of substantially anhydrous hydrofluoric acid as the catalyst at a temperature ranging from 250 to 350° F. at a pressure sufficient to maintain liquid phase conditions, agitating the mixture continuously to insure intimate contacting and prevent separation of liquid phases, continuing the reaction until said wax has reacted with said cyclic hydrocarbon to produce cyclo-alkyl hydrocarbons consisting of cyclic nuclei with attached alkyl groups, separating the reaction mixture into two liquid phases, namely an acid phase and a hydrocarbon phase, separately withdrawing said phases, and recovering from the hydrocarbon phase said cyclo-alkyl hydrocarbons.

FREDERICK E. FREY.